



US011561483B2

(12) **United States Patent**  
**Sasaki et al.**

(10) **Patent No.:** **US 11,561,483 B2**  
(45) **Date of Patent:** **Jan. 24, 2023**

(54) **ELECTROSTATIC CHARGE IMAGE DEVELOPING CARRIER, ELECTROSTATIC CHARGE IMAGE DEVELOPER, AND IMAGE FORMING APPARATUS**

(71) Applicant: **FUJIFILM Business Innovation Corp.**, Tokyo (JP)

(72) Inventors: **Kazutsuma Sasaki**, Minamiashigara (JP); **Yasuo Kadokura**, Minamiashigara (JP); **Shintaro Anno**, Minamiashigara (JP); **Satoshi Miura**, Minamiashigara (JP); **Jumpei Iwasaki**, Minamiashigara (JP)

(73) Assignee: **FUJIFILM Business Innovation Corp.**, Tokyo (JP)

(\*) Notice: Subject to any disclaimer, the term of this patent is extended or adjusted under 35 U.S.C. 154(b) by 0 days.

(21) Appl. No.: **16/945,098**

(22) Filed: **Jul. 31, 2020**

(65) **Prior Publication Data**

US 2021/0271180 A1 Sep. 2, 2021

(30) **Foreign Application Priority Data**

Feb. 28, 2020 (JP) ..... JP2020-034175

(51) **Int. Cl.**

**G03G 9/113** (2006.01)  
**G03G 15/08** (2006.01)  
**G03G 9/08** (2006.01)  
**G03G 9/107** (2006.01)

(52) **U.S. Cl.**

CPC ..... **G03G 9/1131** (2013.01); **G03G 9/0819** (2013.01); **G03G 9/1075** (2013.01); **G03G 9/1139** (2013.01); **G03G 15/08** (2013.01)

(58) **Field of Classification Search**

CPC .. G03G 9/1075; G03G 9/0839; G03G 9/1131; G03G 9/0819; G03G 9/0825; G03G 9/08755; G03G 9/09725  
USPC ..... 430/111.35

See application file for complete search history.

(56) **References Cited**

**U.S. PATENT DOCUMENTS**

5,663,027 A \* 9/1997 Kohri ..... G03G 9/10884  
430/111.4  
6,406,826 B1 6/2002 Suzuki et al.  
9,726,998 B1 \* 8/2017 Morooka ..... G03G 9/09716  
2013/0065175 A1 3/2013 Sakata et al.  
(Continued)

**FOREIGN PATENT DOCUMENTS**

JP 2001-188388 A 7/2001  
JP 2013-061511 A 4/2013  
JP 2018-066892 A 4/2018

*Primary Examiner* — Peter L Vajda

*Assistant Examiner* — Boone Alexander Evans

(74) *Attorney, Agent, or Firm* — Sughrue Mion, PLLC

(57) **ABSTRACT**

An electrostatic charge image developing carrier includes: magnetic particles; and a resin layer coating the magnetic particles and containing inorganic particles, in which an exposed area ratio of the magnetic particles is 0.1% or more and 4.0% or less, an average particle diameter of the inorganic particles is 5 nm or more and 90 nm or less, and a ratio B/A of a surface area B of the electrostatic charge image developing carrier to a plan view area A of the electrostatic charge image developing carrier is 1.020 or more and 1.100 or less when a surface of the electrostatic charge image developing carrier is three-dimensionally analyzed.

**12 Claims, 2 Drawing Sheets**



(56)

**References Cited**

U.S. PATENT DOCUMENTS

2018/0113393 A1 4/2018 Seki et al.  
2018/0143557 A1\* 5/2018 Ueda ..... G03G 9/0821

\* cited by examiner

FIG. 1



FIG.2



**ELECTROSTATIC CHARGE IMAGE  
DEVELOPING CARRIER, ELECTROSTATIC  
CHARGE IMAGE DEVELOPER, AND IMAGE  
FORMING APPARATUS**

**CROSS-REFERENCE TO RELATED  
APPLICATIONS**

This application is based on and claims a priority under 35 USC 119 from Japanese Patent Application No. 2020-034175 filed on Feb. 28, 2020.

**BACKGROUND**

**Technical Field**

The present invention relates to an electrostatic charge image developing carrier, an electrostatic charge image developer, and an image forming apparatus.

**Related Art**

Patent Literature 1 discloses a carrier for electrostatic latent image developer containing magnetic core material particles and a coating layer coating the surface of the core material particles, in which the coating layer contains two or more types of inorganic fine particles, at least one of the two or more types of inorganic fine particles are inorganic fine particles A having conductivity and having a peak particle diameter of 300 nm to 1000 nm, and (BET specific surface area of carrier—BET specific surface area of core material particles) is 1.10 m<sup>2</sup>/g to 1.90 m<sup>2</sup>/g.

Patent Literature 2 discloses an electrostatic latent image developing carrier which is a carrier for electrostatic charge image developer including a coating layer containing a binder resin and fine particles on a core material, in which an area ratio of the exposed core material on the surface of carrier particles is 0.1% or more and 5.0% or less, a maximum exposed area of the exposed core material is 0.03% or less of the surface area of the core material, and the fine particles are contained in 100 parts by weight or more and 500 parts by weight or less based on 100 parts by weight of the binder resin.

Patent Literature 3 discloses an electrophotographic carrier including a coating film containing a binder resin and particles, in which a specific resistance of the particles is 10<sup>12</sup> Ω·cm or more, and a particle diameter D and a film thickness of the binder resin satisfy 1<D/h<5.

Patent Literature 1: JP-A-2018-066892

Patent Literature 2: JP-A-2013-061511

Patent Literature 3: JP-A-2001-188388

Aspects of certain non-limiting embodiments of the present disclosure relate to an electrostatic charge image developing carrier which contains magnetic particles and a resin layer coating the magnetic particles and containing inorganic particles and prevents a decrease in image density when image formation is repeated, as compared with an electrostatic charge image developing carrier in which an average particle diameter of the inorganic particles is less than 5 nm or more than 90 nm, or an electrostatic charge image developing carrier in which an exposed area ratio of the magnetic particles is less than 0.1% or more than 4.0%, or an electrostatic charge image developing carrier in which a ratio B/A of a surface area B to a plan view area A is less than 1.020 or more than 1.100 when a surface thereof is three-dimensionally analyzed.

Aspects of certain non-limiting embodiments of the present disclosure address the above advantages and/or other advantages not described above. However, aspects of the non-limiting embodiments are not required to address the advantages described above, and aspects of the non-limiting embodiments of the present disclosure may not address advantages described above.

According to an aspect of the present disclosure, there is provided an electrostatic charge image developing carrier containing: magnetic particles; and a resin layer coating the magnetic particles and containing inorganic particles, in which an exposed area ratio of the magnetic particles is 0.1% or more and 4.0% or less, an average particle diameter of the inorganic particles is 5 nm or more and 90 nm or less, and a ratio B/A of a surface area B of the electrostatic charge image developing carrier to a plan view area A of the electrostatic charge image developing carrier is 1.020 or more and 1.100 or less when a surface of the electrostatic charge image developing carrier is three-dimensionally analyzed.

**BRIEF DESCRIPTION OF THE DRAWINGS**

Exemplary embodiment(s) of the present invention will be described in detail based on the following figures, wherein:

FIG. 1 is a schematic configuration diagram illustrating an example of an image forming apparatus according to the exemplary embodiment; and

FIG. 2 is a schematic configuration diagram illustrating an example of a process cartridge that is attached to and detached from an image forming apparatus according to the exemplary embodiment.

Reference numbers and signs in FIG. 1 and FIG. 2 are described below.

1Y, 1M, 1C, 1K: photoconductor (an example of image carrier)

2Y, 2M, 2C, 2K: charging roller (an example of charging unit)

3: exposure device (an example of electrostatic charge image forming unit)

3Y, 3M, 3C, 3K: laser beam

4Y, 4M, 4C, 4K: developing device (an example of developing unit)

5Y, 5M, 5C, 5K: primary transfer roller (an example of primary transfer unit)

6Y, 6M, 6C, 6K: photoconductor cleaning device (an example of cleaning unit)

8Y, 8M, 8C, 8K: toner cartridge

10Y, 10M, 10C, 10K: image forming unit

20: intermediate transfer belt (an example of intermediate transfer body)

22: drive roller

24: support roller

26: secondary transfer roller (an example of secondary transfer unit)

28: fixing device (an example of fixing unit)

30: intermediate transfer body cleaning device

P: recording paper (an example of recording medium)

107: photoconductor (an example of image carrier)

108: charging roller (an example of charging unit)

109: exposure device (an example of electrostatic charge image forming unit)

111: developing device (an example of developing unit)

112: transfer device (an example of transfer unit)

113: photoconductor cleaning device (an example of cleaning unit)

- 115: fixing device (an example of fixing unit)
- 116: mounting rail
- 117: housing
- 118: opening for exposure
- 200: process cartridge
- 300: recording paper (an example of recording medium)

## DETAILED DESCRIPTION

Hereinafter, exemplary embodiments of the present disclosure will be described. These descriptions and Examples illustrate the exemplary embodiment, and do not limit the scope of the exemplary embodiment.

In the present disclosure, a numerical range indicated by “to” indicates a range including the numerical values before and after “to” as a minimum value and a maximum value, respectively.

In the numerical ranges described in stages in the present disclosure, an upper limit or a lower limit described in one numerical range may be replaced with an upper limit or a lower limit of the numerical range described in other stages. Further, in the numerical ranges described in the present disclosure, the upper limit or the lower limit of the numerical range may be replaced with values shown in Examples.

In the present disclosure, the term “step” indicates not only an independent step, and even when a step are not clearly distinguished from other steps, this step is included in the term “step” as long as the intended purpose of the step is achieved.

When an exemplary embodiment is described in the present disclosure with reference to the drawings, the configuration of the exemplary embodiment is not limited to the configuration illustrated in the drawings. In addition, the sizes of the members in each drawing are conceptual, and the relative size relationship between the members is not limited to this.

In the present disclosure, each component may include a plurality of corresponding substances. In the present disclosure, in a case of referring to the amount of each component in the composition, when there are a plurality of substances corresponding to each component in the composition, unless otherwise specified, it refers to the total amount of the plurality of substances present in the composition.

In the present disclosure, each component may include a plurality of corresponding particles. When there are a plurality of types of particles corresponding to each component in the composition, unless otherwise specified, the particle diameter of each component means a value for a mixture of the plurality of types of particles present in the composition.

In the present disclosure, the term “(meth)acryl” means at least one of acryl and methacryl, and the term “(meth)acrylate” means at least one of acrylate and methacrylate.

In the present disclosure, the term “electrostatic charge image developing toner” is also referred to as “toner”, the term “electrostatic charge image developing carrier” is also referred to as “carrier”, and the term “electrostatic charge image developer” is also referred to as “developer”.

<Electrostatic Charge Image Developing Carrier>

The carrier according to the exemplary embodiment is a resin-coated carrier which contains magnetic particles and a resin layer coating the magnetic particles and containing inorganic particles.

In the carrier according to the exemplary embodiment, an exposed area ratio of the magnetic particles is 0.1% or more and 4.0% or less, an average particle diameter of the inorganic particles contained in the resin layer is 5 nm or more and 90 nm or less, and a ratio B/A of a surface area B

to a plan view area A is 1.020 or more and 1.100 or less when a surface thereof is three-dimensionally analyzed.

In the exemplary embodiment, carbon black shall not be inorganic particles.

5 In the exemplary embodiment, the average particle diameter of the inorganic particles contained in the resin layer and the average thickness of the resin layer are determined by the following method.

The carrier is embedded in an epoxy resin and cut with a 10 microtome to prepare a carrier cross section. An SEM image of the carrier cross section taken by a scanning electron microscope (SEM) is taken into an image processing analysis device to perform image analysis. 100 inorganic particles (primary particles) in the resin layer are randomly selected, 15 a circle-equivalent diameter (nm) of each particle is determined, and the circle-equivalent diameters are arithmetically averaged to obtain the average particle diameter (nm) of the inorganic particles. The thickness (μm) of the resin layer is 20 measured by randomly selecting 10 points per one particle of the carrier, 100 carriers are further measured, and the thicknesses are arithmetically averaged to obtain the average thickness (μm) of the resin layer.

In the exemplary embodiment, the exposed area ratio of 25 the magnetic particles on the carrier surface is determined by the following method.

A target carrier and magnetic particles obtained by removing the resin layer from the target carrier are prepared. Examples of a method of removing the resin layer from the 30 carrier include a method of removing a resin layer by dissolving a resin component with an organic solvent, and a method of removing a resin layer by heating to eliminate a resin component at about 800°C. The carrier and the magnetic particles are used as measurement samples, the Fe 35 concentrations (atomic %) on the surfaces of the samples are quantified by XPS, and (Fe concentration of carrier)/(Fe concentration of magnetic particles)×100 is calculated to be the exposed area ratio (%) of the magnetic particles.

In the exemplary embodiment, the ratio B/A is an index 40 for evaluating surface roughness. The ratio B/A is obtained by, for example, the following method.

As a device for three-dimensionally analyzing the surface 45 of the carrier, a scanning electron microscope including four secondary electron detectors (e.g., electron beam three-dimensional roughness analyzer ERA-8900FE manufactured by Elionix Inc.) is used and the analysis is performed as follows. The surface of one carrier particle is magnified 5000 times. The distance between measurement points is set to 0.06 μm, the measurement points are 400 points in the long side direction and 300 points in the short side direction, and a region of 24 μm×18 μm is measured to obtain three-dimensional image data.

For the three-dimensional image data, a limit wavelength 55 of a spline filter, which is a frequency selection filter using a spline function, is set to 12 μm to remove wavelengths having a period of 12 μm or more. As a result, a waviness component on the carrier surface is removed and a roughness component is extracted to obtain a roughness curve.

Further, a cutoff value of a Gaussian high-pass filter, 60 which is a frequency selection filter using a Gaussian function, is set to 2.0 μm to remove wavelengths having a period of 2.0 μm or more. As a result, the wavelength corresponding to convex portions of the magnetic particles exposed on the carrier surface is removed from the roughness curve after spline filter processing, and a roughness curve in which the wavelength component having a period of 2.0 μm or more is removed is obtained.

From the three-dimensional roughness curve data after the filter processing, the surface area B ( $\mu\text{m}^2$ ) of a central region of  $12 \mu\text{m} \times 12 \mu\text{m}$  (plan view area A =  $144 \mu\text{m}^2$ ) is obtained to obtain the ratio B/A. The ratio B/A is calculated for 100 carriers and arithmetically averaged.

In the carrier according to the exemplary embodiment, a decrease in image density when image formation is repeated is prevented. The mechanism is presumed as follows.

In a case where the toner comes into contact with the carrier in the developing device to be frictionally charged, when the charge amount of the toner increases excessively, the amount of the toner moving onto the photoconductor decreases and the image density decreases; on the other hand, when the charge amount of the toner decreases excessively, the adhesive force between the carrier and the toner is lowered, the toner is likely to be scattered outside the developing unit and the image density decreases. This phenomenon is likely to occur when image formation with low image density is repeated in a low-temperature and low-humidity environment (e.g., a temperature of  $10^\circ\text{C}$ . and a relative humidity of 15%) (that is, in a state where the stirring of the developer is repeated in the developing device under an atmosphere in which the charge of the toner is likely to change).

In contrast, it is presumed that when using the carrier in which the exposed area ratio of the magnetic particles, the average particle diameter of the inorganic particles in the resin layer, and the ratio B/A are within the above ranges, an excessive increase or decrease in the charge amount of the toner is prevented due to the following reasons (a) to (c), and as a result, a decrease in image density when the image formation is repeated is prevented.

(a) It is presumed that when the exposed area ratio of the magnetic particles is less than 0.1%, the amount of the charge leaked from an exposed portion of the magnetic particles is excessively small, the frictional charging of the toner by the carrier is accelerated, and the charge amount of the toner increases. From this viewpoint, the exposed area ratio of the magnetic particles is 0.1% or more, preferably 0.3% or more, and more preferably 0.5% or more.

In order to leak the charge from the exposed portion of the magnetic particles, the magnetic particles should be exposed to some extent. However, as the magnetic particles are exposed more, the electrical resistance of the carrier is lowered, and the frictional charging of the toner may not be sufficiently proceeded. It is also presumed that as the magnetic particles are exposed more, mechanical stress on the toner increases, the external additive is embedded in the toner particles, the flowability of the toner decreases, and the charge amount decreases. From this viewpoint, the exposed area ratio of the magnetic particles is 4.0% or less, preferably 3.5% or less, and more preferably 3.0% or less.

The exposed area ratio of the magnetic particles may be controlled by using the amount of the resin used for forming the resin layer, and the larger the amount of the resin with respect to the amount of the magnetic particles is, the smaller the exposed area ratio of the magnetic particles is. In addition, the exposed area ratio of the magnetic particles may be controlled by using production conditions for forming the resin layer. Details will be described later.

(b) It is presumed that when the average particle diameter of the inorganic particles in the resin layer is less than 5 nm or more than 90 nm, fine irregularities are less likely to be formed on the carrier surface, the carrier surface is too flat, and the contact between the carrier and the toner becomes surface contact, and the frictional charging of the toner by the carrier is accelerated. From this viewpoint, the average

particle diameter of the inorganic particles in the resin layer is 5 nm or more and 90 nm or less, preferably 5 nm or more and 70 nm or less, more preferably 5 nm or more and 50 nm or less, and still more preferably 8 nm or more and 50 nm or less.

(c) It is presumed that when the ratio B/A is less than 1.020, the carrier surface is too flat, the contact between the carrier and the toner becomes surface contact, and the frictional charging of the toner by the carrier is accelerated.

10 It is presumed that when the ratio B/A is more than 1.100, the number of irregularities on the carrier surface is relatively large, contact points between the carrier and the toner is relatively increased, and the frictional charging of the toner by the carrier is accelerated. From this viewpoint, the 15 ratio B/A is 1.020 or more and 1.100 or less, preferably 1.040 or more and 1.080 or less, and more preferably 1.040 or more and 1.070 or less.

The ratio B/A may be controlled by using production conditions for forming the resin layer. Details will be 20 described later.

From the viewpoint of preventing a decrease in image density when image formation is repeated, in the carrier according to the exemplary embodiment, the average thickness of the resin layer is preferably 0.6  $\mu\text{m}$  or more and 1.4  $\mu\text{m}$  or less. When the average thickness of the resin layer is 0.6  $\mu\text{m}$  or more, the resin layer is less likely to be peeled off when the image formation is repeated, and thus the exposed area ratio of the magnetic particles is maintained. When the average thickness of the resin layer is 1.4  $\mu\text{m}$  or less, fine 25 irregularities are likely to be formed on the carrier surface by the inorganic particles in the resin layer, and the ratio B/A 30 may be easily controlled within the above range.

From the above viewpoints, the average thickness of the resin layer is more preferably 0.8  $\mu\text{m}$  or more and 1.2  $\mu\text{m}$  or less, and still more preferably 0.8  $\mu\text{m}$  or more and 1.1  $\mu\text{m}$  or less.

The average thickness of the resin layer may be controlled by using the amount of the resin used for forming the resin layer, and the larger the amount of the resin with respect to 40 the amount of the magnetic particles is, the larger the average thickness of the resin layer is.

From the viewpoint of preventing a decrease in image density when image formation is repeated, in the carrier according to the exemplary embodiment, the amount of 45 toluene is preferably 100 ppm or less based on the total amount of the carrier. It is presumed that when the amount of toluene is 100 ppm or less, it is possible to prevent toner external additives from adhering to the toluene eluted on the carrier surface, and to prevent toners from adhering to each 50 other due to volatilized toluene, and as a result, the flowability of the toner and the charge amount of the toner are ensured.

From the above viewpoints, the amount of toluene contained in the carrier according to the exemplary embodiment 55 is preferably smaller, more preferably 20 ppm or less, and still more preferably 10 ppm or less. The amount of toluene contained in the carrier according to the exemplary embodiment is most preferably 0 ppm. Here, ppm is an abbreviation for parts per million and is based on mass.

60 In the exemplary embodiment, the amount of toluene contained in the carrier is determined by the following method.

It is presumed that since the amount of toluene contained in the carrier decreases with time, the amount is measured 65 within 24 hours after the opening of individually packaged unopened products that are within half a year after production.

1 g of the carrier is weighed and added to 20 mL of chloroform to dissolve a resin forming the resin layer. After the resin is dissolved, 5 mL of methanol is added thereto, and the mixture is left in a sealed container for one day. The supernatant liquid after standing is used as a sample, gas chromatography mass spectrometry is performed, and the amount of toluene (ppm) based on the total amount of the carrier is determined.

The amount of toluene contained in the carrier may be reduced by changing the production method for forming the resin layer to a dry production method. Details of the dry production method will be described later.

Hereinafter, the configuration of the carrier according to the exemplary embodiment will be described in detail.

[Magnetic Particles]

The magnetic particles are not particularly limited, and known magnetic particles used as a core material of the carrier are applied. Specific examples of the magnetic particles include: particles of magnetic metals such as iron, nickel and cobalt; particles of magnetic oxides such as ferrite and magnetite; resin-impregnated magnetic particles obtained by impregnating porous magnetic powder with a resin; and magnetic powder-dispersed resin particles prepared by dispersing magnetic powder in a resin. In the exemplary embodiment, the magnetic particles are preferably ferrite particles.

The volume average particle diameter of the magnetic particles is preferably 15  $\mu\text{m}$  or more and 100  $\mu\text{m}$  or less, more preferably 20  $\mu\text{m}$  or more and 80  $\mu\text{m}$  or less, and still more preferably 30  $\mu\text{m}$  or more and 60  $\mu\text{m}$  or less.

The arithmetic average height Ra according to JIS B0601: 2001 of a roughness curve of the magnetic particles is preferably 0.1  $\mu\text{m}$  or more and 1  $\mu\text{m}$  or less, and more preferably 0.2  $\mu\text{m}$  or more and 0.8  $\mu\text{m}$  or less.

The arithmetic average height Ra of the roughness curve of the magnetic particles is obtained by observing the magnetic particles at an appropriate magnification (e.g., a magnification of 1000 times) using a surface profile measurement device (e.g., "Ultra-deep color 3D shape measurement microscope VK-9700" manufactured by Keyence Corporation), obtaining a roughness curve at a cutoff value of 0.08 mm, and extracting, from the roughness curve, a reference length of 10  $\mu\text{m}$  in the direction of the average line. The arithmetic average heights Ra of 100 magnetic particles are arithmetically averaged.

As for the magnetic force of the magnetic particles, the saturation magnetization in a magnetic field of 3000 Oersted is preferably 50 emu/g or more, and more preferably 60 emu/g or more. The measurement of the saturation magnetization is performed by using a vibrating sample magnetic measurement device VSMP10-15 (manufactured by Toei Industry Co., Ltd.). The measurement sample is packed in a cell having an inner diameter of 7 mm and a height of 5 mm and set in the above device. The measurement is performed by applying a magnetic field and sweeping up to 3000 Oersted in the maximum. Then, the applied magnetic field is reduced to create a hysteresis curve on a recording paper. The saturation magnetization, the residual magnetization, and the coercive force are determined from data of the curve.

The volume electric resistance (volume resistivity) of the magnetic particles is preferably  $1 \times 10^5 \Omega\cdot\text{cm}$  or more and  $1 \times 10^9 \Omega\cdot\text{cm}$  or less, and more preferably  $1 \times 10^7 \Omega\cdot\text{cm}$  or more and  $1 \times 10^9 \Omega\cdot\text{cm}$  or less.

The volume electric resistance (Q-cm) of the magnetic particles is measured as follows. Measurement targets are placed flat on a surface of a circular jig, on which an electrode plate having 20  $\text{cm}^2$  is arranged, so as to have a

thickness of 1 mm or more and 3 mm or less to form a layer. The electrode plate having 20  $\text{cm}^2$  is placed thereon to sandwich the layer. In order to eliminate a void between the measurement targets, a load of 4 kg is applied on the electrode plate arranged on the layer, and then the layer thickness (cm) is measured. The two electrodes above and below the layer are connected to an electrometer and a high voltage power supply generator. A high voltage is applied to the two electrodes to cause an electric field of 103.8 V/cm, and a current value (A) flowing at this time is read. The measurement environment is a temperature of 20° C. and a relative humidity of 50%. The calculation equation for the volume electric resistance ( $\Omega\cdot\text{cm}$ ) of the measurement target is as shown in the following equation.

$$R = E \times 20 / (I - I_0) / L$$

In the above equation, R represents the volume electric resistance ( $\Omega\cdot\text{cm}$ ) of the measurement target, E represents an applied voltage (V), I represents the current value (A),  $I_0$  represents a current value (A) at the applied voltage of 0 V, and L represents the layer thickness (cm), respectively. The coefficient 20 represents an area ( $\text{cm}^2$ ) of the electrode plate. [Resin Layer]

Examples of the resin forming the resin layer include: a styrene-acrylic acid copolymer, polyolefin resins such as polyethylene and polypropylene; polyvinyl or polyvinylidene resins such as polystyrene, an acrylic resin, polyacrylonitrile, polyvinyl acetate, polyvinyl alcohol, polyvinyl butyral, polyvinyl chloride, polyvinyl carbazole, polyvinyl ether, and polyvinyl ketone; a vinyl chloride-vinyl acetate copolymer; a straight silicone resin having an organosiloxane bond or a modified product thereof; fluororesins such as polytetrafluoroethylene, polyvinyl fluoride, polyvinylidene fluoride, and polychlorotrifluoroethylene; polyester; polyurethane; polycarbonate; amino resins such as a urea-formaldehyde resin; and epoxy resins.

The resin layer preferably contains an acrylic resin having an alicyclic structure. A polymerization component of the acrylic resin having an alicyclic structure is preferably a lower alkyl ester of (meth)acrylic acid (e.g., alkyl (meth)acrylate containing an alkyl group having 1 or more and 9 or less carbon atoms), and specific examples thereof include methyl (meth)acrylate, ethyl (meth)acrylate, propyl (meth)acrylate, butyl (meth)acrylate, hexyl (meth)acrylate, cyclohexyl (meth)acrylate, and 2-ethylhexyl (meth)acrylate. These monomers may be used alone or in combination of two or more thereof.

The acrylic resin having an alicyclic structure preferably contains cyclohexyl (meth)acrylate as a polymerization component. The content of monomer units derived from cyclohexyl (meth)acrylate contained in the acrylic resin having an alicyclic structure is preferably 75 mass % or more and 100 mass % or less, more preferably 85 mass % or more and 100 mass % or less, and still more preferably 95 mass % or more and 100 mass % or less, based on the total mass of the acrylic resin having an alicyclic structure.

Examples of the inorganic particles contained in the resin layer include: particles of metal oxides such as silica, titanium oxide, zinc oxide, and tin oxide; particles of metal compounds such as barium sulfate, aluminum borate, and potassium titanate; and particles of metals such as gold, silver, and copper. Among these, silica particles are preferred from the viewpoints of preventing the toner from blowing out and maintaining the transferability of the toner image.

The surface of the inorganic particles may be subjected to a hydrophobic treatment. Examples of a hydrophobic treat-

ment agent include known organosilicon compounds having an alkyl group (e.g., a methyl group, an ethyl group, a propyl group, and a butyl group), and specific examples thereof include an alkoxysilane compound, a siloxane compound, and a silazane compound. Among these, the hydrophobic treatment agent is preferably a silazane compound, and more preferably hexamethyldisilazane. The hydrophobic treatment agent may be used alone or in combination of two or more thereof.

Examples of a method of subjecting the inorganic particles to a hydrophobic treatment with a hydrophobic treatment agent include: a method of dissolving a hydrophobic treatment agent in supercritical carbon dioxide by using supercritical carbon dioxide and adhering the hydrophobic treatment agent to the surface of the inorganic particles; a method of applying (e.g., spraying or coating) a solution containing a hydrophobic treatment agent and a solvent that dissolves the hydrophobic treatment agent to the surface of the inorganic particles in the atmosphere and adhering the hydrophobic treatment agent to the surfaces of the inorganic particles; and a method of adding a solution containing a hydrophobic treatment agent and a solvent that dissolves the hydrophobic treatment agent to an inorganic particle dispersion liquid and holding the mixed solution in the atmosphere, and then drying the mixed solution containing the inorganic particle dispersion liquid and the solution.

The content of the inorganic particles contained in the resin layer is preferably 10 mass % or more and 60 mass % or less, more preferably 15 mass % or more and 55 mass % or less, and still more preferably 20 mass % or more and 50 mass % or less, based on the total mass of the resin layer.

The content of the silica particles contained in the resin layer is preferably 10 mass % or more and 60 mass % or less, more preferably 15 mass % or more and 55 mass % or less, and still more preferably 20 mass % or more and 50 mass % or less, based on the total mass of the resin layer.

The resin layer may contain conductive particles for the purpose of controlling charging and resistance. Examples of the conductive particles include carbon black and particles having conductivity among the above-mentioned inorganic particles.

Examples of a method of forming the resin layer on the surface of the magnetic particles include a wet production method and a dry production method. The wet production method is a production method using a solvent that dissolves or disperses the resin forming the resin layer. On the other hand, the dry production method is a production method which does not use the solvent.

Examples of the wet production method include: an immersion method of coating by immersing magnetic particles in a resin layer forming resin liquid; a spray method of spraying a resin layer forming resin liquid onto the surface of magnetic particles; a fluidized bed method of spraying a resin layer forming resin liquid with magnetic particles fluidized in a fluidized bed; and a kneader coater method of mixing magnetic particles and a resin layer forming resin liquid in a kneader coater and removing a solvent. These production methods may be repeated or combined.

The resin layer forming resin liquid for use in the wet production method is prepared by dissolving or dispersing a resin and other components in a solvent. The solvent is not particularly limited as long as it dissolves or disperses a resin, and examples thereof include: aromatic hydrocarbons such as toluene and xylene; ketones such as acetone and methyl ethyl ketone; and ethers such as tetrahydrofuran and dioxane.

Examples of the dry production method include a method of heating a mixture of magnetic particles and a resin layer forming resin in a dry state to form a resin layer. Specifically, for example, magnetic particles and a resin layer forming resin are mixed in a gas phase and heated and melted to form a resin layer.

From the viewpoint of reducing the amount of toluene contained in the carrier, the dry production method is preferable to the wet production method.

10 Hereinafter, a dry coating method, which is an exemplary embodiment of the dry production method, will be described.

The dry coating method is a method of forming a resin layer by adhering resin particles to the surface of the magnetic particles to be coated, thereafter applying a mechanical impact force, and melting or softening the resin particles adhered to the surface of the magnetic particles. Specifically, a mixture containing magnetic particles, resin particles and inorganic particles is charged into a high-speed stirring mixer that generates a mechanical impact force, and is subjected to high-speed stirring under no heating or under heating to repeatedly apply an impact force to the mixture. The time for applying the impact force is preferably in the range of 20 minutes or longer and 60 minutes or shorter.

When or after producing the resin-coated carrier by the above method, it is preferable to expose the magnetic particles by, for example, peeling off a part of the resin layer by applying mechanical stress to the resin-coated carrier. For example, when the time for applying the mechanical impact force gets longer, the resin on the surface of the convex portion of the resin-coated carrier may be moved to the concave portion to expose the magnetic particles on the convex portion. In addition, when the produced resin-coated carrier is stirred with a turbuler, a ball mill, a vibration mill or the like, a part of the resin layer may be peeled off to expose the magnetic particles.

In the dry coating method, the step of applying an mechanical impact force using a stirring mixer (referred to as "stirring step") is performed in two steps, and the ratio B/A and the exposed area ratio of the magnetic particles may be controlled by using the temperature in the stirring mixer, the stirring speed, and the stirring duration in each of the first stirring step and the second stirring step.

The ratio B/A tends to decrease and the exposed area ratio of the magnetic particles tends to decrease as the temperature in the stirring mixer rises.

The ratio B/A tends to decrease and the exposed area ratio of the magnetic particles tends to increase as the stirring speed increases.

The ratio B/A tends to decrease and the exposed area ratio of the magnetic particles tends to increase as the stirring duration gets longer.

55 The ratio B/A and the exposed area ratio of the magnetic particles vary particularly depending on the temperature, the stirring speed, and the stirring duration in the second stirring step.

The volume average particle diameter of the carrier is 60 preferably 10  $\mu\text{m}$  or more and 120  $\mu\text{m}$  or less, more preferably 20  $\mu\text{m}$  or more and 100  $\mu\text{m}$  or less, and still more preferably 30  $\mu\text{m}$  or more and 80  $\mu\text{m}$  or less.

<Electrostatic Charge Image Developer>

65 The developer according to the exemplary embodiment is a two-component developer containing the carrier according to the exemplary embodiment and a toner. The toner contains toner particles and, if necessary, an external additive.

## 11

The mixing ratio (mass ratio) of the carrier and the toner in the developer is preferably carrier:toner=100:1 to 100:30, and more preferably 100:3 to 100:20.

## [Toner Particles]

The toner particles contain, for example, a binder resin, and if necessary, a colorant, a release agent, and other additives.

## —Binder Resin—

Examples of the binder resin include vinyl-based resins obtained from a homopolymer of monomers such as styrenes (such as styrene, parachlorostyrene, and  $\alpha$ -methylstyrene), (meth)acrylates (such as methyl acrylate, ethyl acrylate, n-propyl acrylate, n-butyl acrylate, lauryl acrylate, 2-ethylhexyl acrylate, methyl methacrylate, ethyl methacrylate, n-propyl methacrylate, lauryl methacrylate, and 2-ethylhexyl methacrylate), ethylenically unsaturated nitriles (such as acrylonitrile and methacrylonitrile), vinyl ethers (such as vinyl methyl ether and vinyl isobutyl ether), vinyl ketones (such as vinyl methyl ketone, vinyl ethyl ketone, and vinyl isopropenyl ketone), and olefins (such as ethylene, propylene, and butadiene), or a copolymer combining two or more of these monomers.

Examples of the binder resin also include non-vinyl-based resins such as an epoxy resin, a polyester resin, a polyurethane resin, a polyamide resin, a cellulose resin, a polyether resin, and a modified rosin, a mixture of these non-vinyl-based resins and the vinyl-based resins, or a graft polymer obtained by polymerizing a vinyl-based monomer in the coexistence of these non-vinyl-based resins.

These binder resins may be used alone or in combination of two or more thereof.

The binder resin is preferably a polyester resin.

Examples of the polyester resin include known amorphous polyester resins. As the polyester resin, a crystalline polyester resin may be used in combination with the amorphous polyester resin. However, the content of the crystalline polyester resin is preferably 2 mass % or more and 40 mass % or less, and more preferably 2 mass % or more and 20 mass % or less, based on the entire binder resin.

The “crystalline” of a resin refers to having a clear endothermic peak in differential scanning calorimetry (DSC), not a stepwise change in endothermic amount, and specifically refers to that the half-value width of the endothermic peak when measured at a temperature rising rate of 10 ( $^{\circ}$  C./min) is within 10 $^{\circ}$  C.

On the other hand, the “amorphous” of the resin refers to that the half-value width is larger than 10 $^{\circ}$  C., that the endothermic amount changes stepwise, or that no clear endothermic peak is observed.

## Amorphous Polyester Resin

Examples of the amorphous polyester resin include a polycondensate of a polycarboxylic acid and a polyhydric alcohol. As the amorphous polyester resin, a commercially available product or a synthesized product may be used.

Examples of the polycarboxylic acid include aliphatic dicarboxylic acids (such as oxalic acid, malonic acid, maleic acid, fumaric acid, citraconic acid, itaconic acid, glutaconic acid, succinic acid, alkeneysuccinic acid, adipic acid, and sebacic acid), alicyclic dicarboxylic acids (such as cyclohexanedicarboxylic acid), aromatic dicarboxylic acids (such as terephthalic acid, isophthalic acid, phthalic acid, and naphthalenedicarboxylic acid), and an anhydride or a lower alkyl ester (e.g., having 1 or more and 5 or less carbon atoms) thereof. Among these, the polycarboxylic acid is preferably, for example, an aromatic dicarboxylic acid.

As the polycarboxylic acid, a tricarboxylic acid or higher carboxylic acid having a cross-linked structure or a branched

## 12

structure may be used in combination with a dicarboxylic acid. Examples of the tricarboxylic acid or higher carboxylic acid include trimellitic acid, pyromellitic acid, and an anhydride or a lower alkyl ester (e.g., having 1 or more and 5 or less carbon atoms) thereof.

The polycarboxylic acid may be used alone or in combination of two or more thereof.

Examples of the polyhydric alcohol include aliphatic diols (such as ethylene glycol, diethylene glycol, triethylene glycol, propylene glycol, butanediol, hexanediol, and neopentyl glycol), alicyclic diols (such as cyclohexanediol, cyclohexanediethanol, and hydrogenated bisphenol A), and aromatic diols (such as a bisphenol A ethylene oxide adduct and a bisphenol A propylene oxide adduct). Among these, the polyhydric alcohol is preferably, for example, an aromatic diol and an alicyclic diol, and more preferably an aromatic diol.

As the polyhydric alcohol, a trihydric alcohol or higher polyhydric alcohol having a cross-linked structure or a branched structure may be used in combination with a diol. Examples of the trihydric alcohol or higher polyhydric alcohol include glycerin, trimethylolpropane, and pentaerythritol.

The polyhydric alcohol may be used alone or in combination of two or more thereof.

The glass transition temperature ( $T_g$ ) of the amorphous polyester resin is preferably 50 $^{\circ}$  C. or higher and 80 $^{\circ}$  C. or lower, and more preferably 50 $^{\circ}$  C. or higher and 65 $^{\circ}$  C. or lower.

The glass transition temperature is obtained from a DSC curve obtained by differential scanning calorimetry (DSC), and is more specifically obtained by the “extrapolated glass transition onset temperature” described in JIS K 7121:1987 “Method for measuring glass transition temperature of plastics”, which is a method for obtaining the glass transition temperature.

The weight average molecular weight ( $M_w$ ) of the amorphous polyester resin is preferably 5,000 or more and 1,000,000 or less, and more preferably 7,000 or more and 500,000 or less.

The number average molecular weight ( $M_n$ ) of the amorphous polyester resin is preferably 2,000 or more and 100,000 or less.

The molecular weight distribution  $M_w/M_n$  of the amorphous polyester resin is preferably 1.5 or more and 100 or less, and more preferably 2 or more and 60 or less.

The weight average molecular weight and the number average molecular weight are measured by gel permeation chromatography (GPC). The molecular weight is measured by GPC by using a GPC HLC-8120GPC manufactured by Tosoh Corporation as a measurement device, a column TSKgel Super HM-M (15 cm) manufactured by Tosoh Corporation, and a THF solvent. The weight average molecular weight and the number average molecular weight are calculated from the measurement result using a molecular weight calibration curve prepared using a monodispersed polystyrene standard sample.

The amorphous polyester resin is obtained by a well-known production method. Specifically, for example, the amorphous polyester resin may be obtained by a method in which the polymerization temperature is set to 180 $^{\circ}$  C. or higher and 230 $^{\circ}$  C. or lower, the pressure in the reaction system is reduced as necessary, and the reaction is performed while removing water and alcohol generated during the condensation.

When raw material monomers are insoluble or incompatible at the reaction temperature, a high boiling point solvent

may be added as a dissolution assisting agent for dissolution. In this case, the polycondensation reaction is carried out while distilling off the dissolution assisting agent. When there is a poorly compatible monomer in the copolymerization reaction, it is preferable that the poorly compatible monomer is firstly condensed with an acid or alcohol to be polycondensed with the poorly compatible monomer and then the obtained product is polycondensed with the main component.

#### Crystalline Polyester Resin

Examples of the crystalline polyester resin include a polycondensate of a polycarboxylic acid and a polyhydric alcohol. As the crystalline polyester resin, a commercially available product or a synthesized product may be used.

Here, in order to easily form a crystal structure, the crystalline polyester resin is preferably a polycondensate using a polymerizable monomer having a linear aliphatic group rather than a polymerizable monomer having an aromatic ring.

Examples of the polycarboxylic acid include aliphatic dicarboxylic acids (such as oxalic acid, succinic acid, glutaric acid, adipic acid, suberic acid, azelaic acid, sebacic acid, 1,9-nonanedicarboxylic acid, 1,10-decanedicarboxylic acid, 1,12-dodecanedicarboxylic acid, 1,14-tetradecanedi-carboxylic acid, and 1,18-octadecanedicarboxylic acid), aromatic dicarboxylic acids (e.g., dibasic acids such as phthalic acid, isophthalic acid, terephthalic acid, and naphthalene-2, 6-dicarboxylic acid), and an anhydride or a lower alkyl ester (e.g., having 1 or more and 5 or less carbon atoms) thereof.

As the polycarboxylic acid, a tricarboxylic acid or higher carboxylic acid having a cross-linked structure or a branched structure may be used in combination with a dicarboxylic acid. Examples of the tricarboxylic acid include aromatic carboxylic acids (such as 1,2,3-benzenetricarboxylic acid, 1,2,4-benzenetricarboxylic acid, and 1,2,4-naphthalenetri-carboxylic acid), and an anhydride or a lower alkyl ester (e.g., having 1 or more and 5 or less carbon atoms) thereof.

As the polycarboxylic acid, a dicarboxylic acid having a sulfonic acid group or a dicarboxylic acid having an ethylenic double bond may be used in combination with these dicarboxylic acids.

The polycarboxylic acid may be used alone or in combination of two or more thereof.

Examples of the polyhydric alcohol include aliphatic diols (such as a linear aliphatic diol having 7 or more and 20 or less carbon atoms in the main chain portion). Examples of the aliphatic diol include ethylene glycol, 1,3-propanediol, 1,4-butanediol, 1,5-pentanediol, 1,6-hexanediol, 1,7-heptanediol, 1,8-octanediol, 1,9-nonanediol, 1,10-decanediol, 1,11-undecanediol, 1,12-dodecanediol, 1,13-tridecanediol, 1,14-tetradecanediol, 1,18-octadecanediol, and 1,14-eicosanediol. Among these, the aliphatic diol is preferably 1,8-octanediol, 1,9-nonanediol, and 1,10-decanediol.

As the polyhydric alcohol, a trihydric alcohol or higher alcohol having a cross-linked structure or a branched structure may be used in combination with a diol. Examples of the trihydric alcohol or higher polyhydric alcohol include glycerin, trimethylolethane, trimethylolpropane, and pentaerythritol.

The polyhydric alcohol may be used alone or in combination of two or more thereof.

Here, the polyhydric alcohol preferably has an aliphatic diol content of 80 mol % or more, and preferably 90 mol % or more.

The melting temperature of the crystalline polyester resin is preferably 50° C. or higher and 100° C. or lower, more

preferably 55° C. or higher and 90° C. or lower, and still more preferably 60° C. or higher and 85° C. or lower.

The melting temperature is obtained from the DSC curve obtained by differential scanning calorimetry (DSC) according to the "melting peak temperature" described in JIS K 7121:1987 "Method for measuring transition temperature of plastics", which is a method for obtaining the melting temperature.

The weight average molecular weight (Mw) of the crystalline polyester resin is preferably 6,000 or more and 35,000 or less.

The crystalline polyester resin may be obtained by a well-known production method, similar to the amorphous polyester resin.

The content of the binder resin is preferably 40 mass % or more and 95 mass % or less, more preferably 50 mass % or more and 90 mass % or less, and still more preferably 60 mass % or more and 85 mass % or less, based on the total toner particles.

#### —Colorant—

Examples of the colorant include: pigments such as Carbon Black, Chrome Yellow, Hansa Yellow, Benzidine Yellow, Slene Yellow, Quinoline Yellow, Pigment Yellow, Permanent Orange GTR, Pyrazolone Orange, Balkan Orange, Watch Young Red, Permanent Red, Brilliant Carmine 3B, Brilliant Carmine 6B, DuPont Oil Red, Pyrazolone Red, Resole Red, Rhodamine B Lake, Lake Red C, Pigment Red, Rose Bengal, Aniline Blue, Ultramarine Blue, Chalco oil Blue, Methylene Blue Chloride, Phthalocyanine Blue, Pigment Blue, Phthalocyanine Green, and Malachite Green Oxalate; and acridine, xanthene, azo, benzoquinone, azine, anthraquinone, thioindigo, dioxazine, thiazine, azomethine, indigo, phthalocyanine, aniline black, polymethine, triphenylmethane, diphenylmethane, and thiazole dyes.

The colorants may be used alone or in combination of two or more thereof.

As the colorant, a surface-treated colorant may be used as necessary, or the colorant may be used in combination with a dispersant. In addition, a plurality of types of colorants may be used in combination.

The content of the colorant is preferably 1 mass % or more and 30 mass % or less, and more preferably 3 mass % or more and 15 mass % or less, based on the total toner particles.

#### —Release Agent—

Examples of the release agent include: hydrocarbon wax; natural wax such as carnauba wax, rice wax, and candelilla wax; synthetic wax or mineral or petroleum wax such as montan wax; and ester wax such as fatty acid ester and montanic acid ester. The release agent is not particularly limited thereto.

The melting temperature of the release agent is preferably 50° C. or higher and 110° C. or lower, and more preferably 60° C. or higher and 100° C. or lower.

The melting temperature is obtained from the DSC curve obtained by differential scanning calorimetry (DSC) according to the "melting peak temperature" described in JIS K 7121:1987 "Method for measuring transition temperature of plastics", which is a method for obtaining the melting temperature.

The content of the release agent is preferably 1 mass % or more and 20 mass % or less, and more preferably 5 mass % or more and 15 mass % or less, based on the total toner particles.

## —Other Additives—

Examples of other additives include known additives such as magnetic materials, charge control agents, and inorganic powders. These additives are contained in the toner particles as internal additives.

## —Characteristics of Toner Particles—

The toner particles may be toner particles having a single-layer structure, or so-called core-shell structure toner particles (core-shell type particles) composed of a core portion (core particles) and a coating layer (shell layer) for coating the core portion.

The core-shell structure toner particles preferably include, for example, a core portion containing a binder resin and, if necessary, other additives such as a colorant and a release agent, and a coating layer containing the binder resin.

The volume average particle diameter  $D_{50v}$  of the toner particles is preferably 2  $\mu\text{m}$  or more and 10  $\mu\text{m}$  or less, and more preferably 4  $\mu\text{m}$  or more and 8  $\mu\text{m}$  or less.

The volume average particle diameter  $D_{50v}$  of the toner particles is measured using a Coulter Multisizer II (manufactured by Beckman Coulter, Inc.) and the electrolytic solution is ISOTON-II (manufactured by Beckman Coulter, Inc.).

In the measurement, 0.5 mg or more and 50 mg or less of a measurement sample is added to 2 ml of a 5 mass % aqueous solution of a surfactant (preferably sodium alkylbenzenesulfonate) as a dispersant. The obtained mixture is added to 100 ml or more and 150 ml or less of the electrolytic solution.

The electrolytic solution in which the sample is suspended is subjected to a dispersion treatment for 1 minute with an ultrasonic disperser, and the Coulter Multisizer II is used to measure the particle diameter distribution of particles having a particle diameter in the range of 2  $\mu\text{m}$  or more and 60  $\mu\text{m}$  or less using an aperture having an aperture diameter of 100  $\mu\text{m}$ . The number of the particles sampled is 50,000. With respect to the measured particle diameter, a cumulative distribution by volume drawn from the side of the small diameter, and the particle diameter corresponding to the cumulative percentage of 50% is defined as the volume average particle diameter  $D_{50v}$ .

The average circularity of the toner particles is preferably 0.94 or more and 1.00 or less, and more preferably 0.95 or more and 0.98 or less.

The average circularity of the toner particles is obtained according to (circle equivalent perimeter)/(perimeter), that is, (perimeter of circle having the same projected area as the particle image)/(perimeter of particle projection image). Specifically, the average circularity of the toner particles is a value measured by the following method.

First, the toner particles as measurement targets are suctioned and collected to form a flat flow, and flash light is emitted instantly to capture a particle image as a still image. The particle image is determined by a flow type particle image analyzer (FPIA-3000 manufactured by Sysmex Corporation) for image analysis. The number of the toner particles sampled for determining the average circularity is 3,500.

When the toner contains an external additive, the toner (developer) as a measurement target is dispersed in water containing a surfactant, then an ultrasonic treatment is performed to obtain toner particles from which the external additive has been removed.

## —Method for Producing Toner Particles—

The toner particles may be produced by either a dry production method (e.g., a kneading pulverization method) or a wet production method (e.g., an aggregation and coales-

cence method, a suspension polymerization method, and a dissolution suspension method). These production methods are not particularly limited and known production methods are adopted. Among these, the toner particles are preferably obtained by the aggregation and coalescence method.

Specifically, in the case of producing the toner particles by the aggregation and coalescence method, the toner particles are produced by, for example, a step of preparing a resin particle dispersion liquid in which binder resin particles are dispersed (resin particle dispersion liquid preparation step), a step of aggregating resin particles and if necessary other particles in the resin particle dispersion liquid or in a dispersion liquid after mixing other particle dispersion liquids if necessary, to form aggregated particles (aggregated particle forming step), and a step of heating an aggregated particle dispersion liquid in which the aggregated particles are dispersed to fuse and coalesce the aggregated particles to form toner particles (fusion and coalesce step).

Hereinafter, the details of each step will be described.

In the following description, a method for obtaining toner particles containing a colorant and a release agent will be described, but the colorant and the release agent are used as necessary. Of course, other additives other than the colorant and the release agent may be used.

## —Resin Particle Dispersion Liquid Preparation Step—

A colorant particle dispersion liquid in which colorant particles are dispersed and a release agent particle dispersion liquid in which release agent particles are dispersed are prepared together with a resin particle dispersion liquid in which binder resin particles are dispersed.

The resin particle dispersion liquid is prepared, for example, by dispersing resin particles in a dispersion medium with a surfactant.

Examples of the dispersion medium for use in the resin particle dispersion liquid include an aqueous medium.

Examples of the aqueous medium include water such as distilled water and ion-exchanged water, and alcohols. The aqueous medium may be used alone or in combination of two or more thereof.

Examples of the surfactant include: sulfate ester salt-based, sulfonate-based, phosphate ester-based, and soap-based anionic surfactants; amine salt-based and quaternary ammonium salt-based cationic surfactants; and polyethylene glycol-based, alkylphenol ethylene oxide adduct-based, and polyhydric alcohol-based nonionic surfactants. Among these, anionic surfactants and cationic surfactants are particularly preferred. The nonionic surfactant may be used in combination with an anionic surfactant or a cationic surfactant.

The surfactant may be used alone or in combination of two or more thereof.

For the resin particle dispersion liquid, examples of a method of dispersing the resin particles in the dispersion medium include general dispersion methods using a rotary shearing homogenizer, a ball mill having a media, a sand mill, and a dyno mill, or the like. Depending on the type of the resin particles, the resin particles may be dispersed in the dispersion medium by using a phase inversion emulsification method. The phase inversion emulsification method is a method of dispersing a resin in an aqueous medium in the form of particles by dissolving a resin to be dispersed in a hydrophobic organic solvent in which the resin is soluble, adding a base to the organic continuous phase (O phase) for neutralization, and then adding an aqueous medium (W phase) to change the phase from W/O to O/W.

The volume average particle diameter of the resin particles dispersing in the resin particle dispersion liquid is

preferably, for example, 0.01  $\mu\text{m}$  or more and 1  $\mu\text{m}$  or less, more preferably 0.08  $\mu\text{m}$  or more and 0.8  $\mu\text{m}$  or less, and still more preferably 0.1  $\mu\text{m}$  or more and 0.6  $\mu\text{m}$  or less.

Regarding the volume average particle diameter of the resin particles, a cumulative distribution by volume is drawn from the side of the smallest diameter with respect to particle diameter ranges (so-called channels) separated using the particle diameter distribution obtained by the measurement of a laser diffraction-type particle diameter distribution measurement device (e.g., LA-700 manufactured by Horiba, Ltd.), and a particle diameter corresponding to the cumulative percentage of 50% with respect to the entire particles is set as a volume average particle diameter  $D_{50v}$ . The volume average particle diameter of the particles in other dispersion liquids is measured in the same manner.

The content of the resin particles contained in the resin particle dispersion liquid is preferably 5 mass % or more and 50 mass % or less, and more preferably 10 mass % or more and 40 mass % or less.

For example, the colorant particle dispersion liquid and the release agent particle dispersion liquid are prepared in the same manner as the resin particle dispersion liquid. That is, regarding the volume average particle diameter of particles, the dispersion medium, the dispersion method, and the content of the particles in the resin particle dispersion liquid, the same applies to the colorant particles dispersed in the colorant particle dispersion liquid and the release agent particles dispersed in the release agent particle dispersion liquid.

#### —Aggregated Particle Forming Step—

Next, the resin particle dispersion liquid, the colorant particle dispersion liquid, and the release agent particle dispersion liquid are mixed.

Then, in the mixed dispersion liquid, the resin particles, the colorant particles, and the release agent particles are hetero-aggregated to form aggregated particles containing the resin particles, the colorant particles, and the release agent particles, which have a diameter close to the diameter of the target toner particles.

Specifically, for example, an aggregating agent is added to the mixed dispersion liquid, the pH of the mixed dispersion liquid is adjusted to acidic (e.g., a pH of 2 or more and 5 or less), and a dispersion stabilizer is added if necessary. Then, the resin particles are heated to a temperature (specifically, for example, “the glass transition temperature of resin particles-30° C.” or higher and “the glass transition temperature-10° C.” or lower) close to the glass transition temperature to aggregate the particles dispersed in the mixed dispersion liquid, and thus the aggregated particles are formed.

In the aggregated particle forming step, for example, while stirring the mixed dispersion liquid with a rotary shear homogenizer, an aggregating agent is added at room temperature (e.g., 25° C.), the pH of the mixed dispersion liquid is adjusted to acidic (e.g., a pH of 2 or more and 5 or less), and a dispersion stabilizer is added if necessary. Then, the heating may be performed.

Examples of the aggregating agent include a surfactant having a polarity opposite to that of the surfactant contained in the mixed dispersion liquid, an inorganic metal salt, and a divalent or higher metal complex. When a metal complex is used as the aggregating agent, the amount of the surfactant used is reduced and the charging characteristics are improved.

If necessary, an additive that forms a complex or a similar bond with the metal ion of the aggregating agent may be

used in combination with the aggregating agent. A chelating agent is preferably used as the additive.

Examples of the inorganic metal salt include: metal salts such as calcium chloride, calcium nitrate, barium chloride, magnesium chloride, zinc chloride, aluminum chloride, and aluminum sulfate; and inorganic metal salt polymers such as polyaluminum chloride, polyaluminum hydroxide, and calcium polysulfide.

A water-soluble chelating agent may be used as the chelating agent. Examples of the chelating agent include: oxycarboxylic acids such as tartaric acid, citric acid and gluconic acid; and aminocarboxylic acids such as iminodiacetic acid (IDA), nitrilotriacetic acid (NTA), and ethylenediaminetetraacetic acid (EDTA).

The amount of the chelating agent added is preferably 0.01 part by mass or more and 5.0 parts by mass or less, and more preferably 0.1 part by mass or more and less than 3.0 parts by mass, based on 100 parts by mass of the resin particles.

#### —Fusion and Coalesce Step—

Next, the aggregated particle dispersion liquid in which the aggregated particles are dispersed is heated to, for example, a temperature equal to or higher than the glass transition temperature of the resin particles (e.g., a temperature higher than the glass transition temperature of the resin particles by 10° C. to 30° C.) to fuse and coalesce the aggregated particles to form the toner particles.

After the above steps, the toner particles are obtained.

The toner particles may also be produced by a step of forming second aggregated particles by obtaining an aggregated particle dispersion liquid in which aggregated particles are dispersed, and then further mixing the aggregated particle dispersion liquid and a resin particle dispersion liquid in which resin particles are dispersed to further adhere and aggregate the resin particles to the surface of the aggregated particles, and a step of forming core-shell structure toner particles by heating a second aggregated particle dispersion liquid in which the second aggregated particles are dispersed to fuse and coalesce the second aggregated particles.

After the fusion and coalesce step, the toner particles formed in the solution are subjected to known washing step, solid-liquid separation step, and drying step to obtain dried toner particles. In the washing step, from the viewpoint of chargeability, it is preferable to sufficiently perform displacement washing with ion-exchanged water. In the solid-liquid separation step, suction filtration, pressure filtration or the like may be performed from the viewpoint of productivity. In the drying step, freeze-drying, air-flow drying, fluidized drying, vibration-type fluidized drying or the like may be performed from the viewpoint of productivity.

Then, the toner particles according to the exemplary embodiment are produced, for example, by adding an external additive to the obtained dried toner particles and mixing the two. The mixing may be performed by, for example, a V-blender, a Henschel mixer, or a Loedige mixer. Further, if necessary, coarse particles in the toner may be removed using a vibration sieving machine, a wind sieving machine or the like.

#### —External Additive—

Examples of the external additive include inorganic particles. Examples of the inorganic particles include  $\text{SiO}_2$ ,  $\text{TiO}_2$ ,  $\text{Al}_2\text{O}_3$ ,  $\text{CuO}$ ,  $\text{ZnO}$ ,  $\text{SnO}_2$ ,  $\text{CeO}_2$ ,  $\text{Fe}_2\text{O}_3$ ,  $\text{MgO}$ ,  $\text{BaO}$ ,  $\text{CaO}$ ,  $\text{K}_2\text{O}$ ,  $\text{Na}_2\text{O}$ ,  $\text{ZrO}_2$ ,  $\text{CaO} \cdot \text{SiO}_2$ ,  $\text{K}_2\text{O} \cdot (\text{TiO}_2)_n$ ,  $\text{Al}_2\text{O}_3 \cdot 2\text{SiO}_2$ ,  $\text{CaCO}_3$ ,  $\text{MgCO}_3$ ,  $\text{BaSO}_4$ , and  $\text{MgSO}_4$ .

The surface of the inorganic particles as an external additive is preferably subjected to a hydrophobic treatment. The hydrophobic treatment is performed, for example, by

immersing the inorganic particles in a hydrophobic treatment agent. The hydrophobic treatment agent is not particularly limited, and examples thereof include a silane coupling agent, a silicone oil, a titanate coupling agent, and an aluminum coupling agent. The hydrophobic treatment agent may be used alone or in combination of two or more thereof.

The amount of the hydrophobic treatment agent is generally, for example, 1 part by mass or more and 10 parts by mass or less based on 100 parts by mass of the inorganic particles.

Examples of the external additive include resin particles (resin particles of polystyrene, polymethylmethacrylate, and melamine resin), and cleaning activators (such as metal salts of higher fatty acids typified by zinc stearate, and particles of fluoropolymer).

The amount of the external additive is preferably 0.01 mass % or more and 5 mass % or less, and more preferably 0.01 mass % or more and 2.0 mass % or less, based on the toner particles.

<Image Forming Apparatus and Image Forming Method>

The image forming apparatus according to the exemplary embodiment includes: an image carrier; a charging unit for charging the surface of the image carrier; an electrostatic charge image forming unit for forming an electrostatic charge image on the surface of the charged image carrier; a developing unit for developing, as a toner image, the electrostatic charge image formed on the surface of the image carrier by using the electrostatic charge image developer a transfer unit for transferring the toner image formed on the surface of the image carrier onto the surface of a recording medium; and a fixing unit for fixing the toner image transferred on the surface of the recording medium. Then, the electrostatic charge image developer according to the exemplary embodiment is applied as the electrostatic charge image developer.

In the image forming apparatus according to the exemplary embodiment, an image forming method (the image forming method according to the exemplary embodiment) is performed, which includes: a charging step of charging the surface of the image carrier; an electrostatic charge image forming step of forming an electrostatic charge image on the surface of the charged image carrier; a development step of developing, as a toner image, the electrostatic charge image formed on the surface of the image carrier by using the electrostatic charge image developer according to the exemplary embodiment; a transfer step of transferring the toner image formed on the surface of the image carrier onto the surface of the recording medium; and a fixing step of fixing the toner image transferred on the surface of the recording medium.

As the image forming apparatus according to the exemplary embodiment, known image forming apparatuses are applied, for example, a direct transfer type apparatus that directly transfers the toner image formed on the surface of the image carrier onto the recording medium, an intermediate transfer type apparatus that primarily transfers the toner image formed on the surface of the image carrier onto the surface of an intermediate transfer body, and secondarily transfers the toner image transferred on the surface of the intermediate transfer body onto the surface of the recording medium, an apparatus including a cleaning unit for cleaning the surface of the image carrier before the charging after the transfer of the toner image, and an apparatus including a charge removing unit for removing the charge by irradiating the surface of the image carrier before the charging with removing light after the transfer of the toner image.

When the image forming apparatus according to the exemplary embodiment is an intermediate transfer type apparatus, the transfer unit includes, for example, an intermediate transfer body with a toner image transferred onto the surface thereof, a primary transfer unit for primarily transferring the toner image formed on the surface of the image carrier onto the surface of the intermediate transfer body, and a secondary transfer unit for secondarily transferring the toner image transferred on the surface of the intermediate transfer body onto the surface of the recording medium.

In the image forming apparatus according to the exemplary embodiment, for example, a portion including the developing unit may have a cartridge structure (process cartridge) that is attached to and detached from the image forming apparatus. As the process cartridge, for example, a process cartridge including a developing unit for storing the electrostatic charge image developer according to the exemplary embodiment is preferably used.

20 Hereinafter, an example of the image forming apparatus according to the exemplary embodiment will be described, but the image forming apparatus is not limited thereto. In the following description, the main parts shown in the drawings will be described, and description of the other parts will be 25 omitted.

FIG. 1 is a schematic configuration diagram illustrating the image forming apparatus according to the exemplary embodiment.

The image forming apparatus illustrated in FIG. 1 30 includes first to fourth electrophotographic image forming units 10Y, 10M, 10C, and 10K that output images of respective colors of yellow (Y), magenta (M), cyan (C), and black (K) based on image data subjected to color separation. These image forming units (hereinafter, may also be simply 35 referred to as "units") 10Y, 10M, 10C, and 10K are arranged side by side in the horizontal direction with a predetermined distance therebetween. These units 10Y, 10M, 10C, and 10K may be process cartridges that are attached to and detached from the image forming apparatus.

40 Above the units 10Y, 10M, 10C, and 10K, an intermediate transfer belt 20 (an example of the intermediate transfer body) is extended through the units. The intermediate transfer belt 20 is provided around a drive roller 22 and a support roller 24, and is configured to run in the direction from the 45 first unit 10Y to the fourth unit 10K. A force is applied to the support roller 24 in a direction away from the drive roller 22 by a spring or the like (not illustrated), and tension is applied to the intermediate transfer belt 20 wound around the support roller 24 and the drive roller 22. An intermediate transfer body cleaning device 30 is provided on an image carrier side surface of the intermediate transfer belt 20 so as 50 to face the drive roller 22.

Developing devices 4Y, 4M, 4C, and 4K (an example of the developing unit) of the units 10Y, 10M, 10C, and 10K 55 are supplied with yellow, magenta, cyan, and black toners stored in toner cartridges 8Y, 8M, 8C, and 8K, respectively.

Since the first to fourth units 10Y, 10M, 10C, and 10K have the same configuration and operation, here, the first unit 10Y, which is arranged on the upstream side in the 60 running direction of the intermediate transfer belt and forms a yellow image, will be described as a representative.

The first unit 10Y includes a photoconductor 1Y functioning as an image carrier. Around the photoconductor 1Y, the following members are disposed in order: a charging roller 2Y (an example of the charging unit) for charging the surface of the photoconductor 1Y to a predetermined potential; an exposure device 3 (an example of the electrostatic

charge image forming unit) for forming an electrostatic charge image by exposing the charged surface with a laser beam **3Y** based on an image signal subjected to color separation; a developing device **4Y** (an example of the developing unit) for developing the electrostatic charge image by supplying the charged toner to the electrostatic charge image; a primary transfer roller **5Y** (an example of the primary transfer unit) for transferring the developed toner image onto the intermediate transfer belt **20**; and a photoconductor cleaning device **6Y** (an example of the cleaning unit) for removing the toner remaining on the surface of the photoconductor **1Y** after the primary transfer.

The primary transfer roller **5Y** is disposed inside the intermediate transfer belt **20** and is provided at a position facing the photoconductor **1Y**. A bias power source (not illustrated) for applying a primary transfer bias is connected to each of the primary transfer rollers **5Y**, **5M**, **5C**, and **5K** of the respective units. Each bias power source changes the value of the transfer bias applied to each primary transfer roller under the control of a controller (not illustrated).

Hereinafter, the operation of forming a yellow image in the first unit **10Y** will be described.

First, prior to the operation, the surface of the photoconductor **1Y** is charged to a potential of  $-600$  V to  $-800$  V by using the charging roller **2Y**.

The photoconductor **1Y** is formed by laminating a photoconductive layer on a conductive substrate (e.g., having volume resistivity at  $20^\circ$  C. of  $1 \times 10^{-6}$   $\Omega$ cm or less). The photoconductive layer generally has high resistance (resistance of general resin), but, has a property that when irradiated with a laser beam, the specific resistance of the portion irradiated with the laser beam changes. Therefore, the exposure device **3** irradiates the charged surface of the photoconductor **1Y** with the laser beam **3Y** according to yellow image data sent from the controller (not illustrated). Accordingly, an electrostatic charge image having a yellow image pattern is formed on the surface of the photoconductor **1Y**.

The electrostatic charge image is an image formed on the surface of the photoconductor **1Y** by charging, and is a so-called negative latent image formed by lowering the specific resistance of the portion of the photoconductive layer irradiated with the laser beam **3Y** to flow a charge charged on the surface of the photoconductor **1Y** and by, on the other hand, leaving a charge of a portion not irradiated with the laser beam **3Y**.

The electrostatic charge image formed on the photoconductor **1Y** rotates to a predetermined developing position as the photoconductor **1Y** runs. Then, at this developing position, the electrostatic charge image on the photoconductor **1Y** is developed and visualized as a toner image by the developing device **4Y**.

In the developing device **4Y**, for example, an electrostatic charge image developer containing at least a yellow toner and a carrier is stored. The yellow toner is frictionally charged by being stirred in the developing device **4Y**, and has a charge of the same polarity (negative) as the charge charged on the photoconductor **1Y** and is carried on a developer roller (an example of a developer carrier). Then, when the surface of the photoconductor **1Y** passes through the developing device **4Y**, the yellow toner electrostatically adheres to a discharged latent image portion on the surface of the photoconductor **1Y**, and the latent image is developed by the yellow toner. The photoconductor **1Y** on which the yellow toner image is formed continues to run at a prede-

termined speed, and the toner image developed on the photoconductor **1Y** is conveyed to a predetermined primary transfer position.

When the yellow toner image on the photoconductor **1Y** is conveyed to the primary transfer position, a primary transfer bias is applied to the primary transfer roller **5Y**, an electrostatic force from the photoconductor **1Y** to the primary transfer roller **5Y** acts on the toner image, and the toner image on the photoconductor **1Y** is transferred onto the intermediate transfer belt **20**. The transfer bias applied at this time has a polarity (+) opposite to the polarity (-) of the toner, and is controlled to  $+10$   $\mu$ A, for example, by the controller (not illustrated) in the first unit **10Y**.

On the other hand, the toner remaining on the photoconductor **1Y** is removed and collected by the photoconductor cleaning device **6Y**.

The primary transfer bias applied to the primary transfer rollers **5M**, **5C**, and **5K** at and after the second unit **10M** is also controlled similar to the first unit.

In this way, the intermediate transfer belt **20** onto which the yellow toner image is transferred by the first unit **10Y** is sequentially conveyed through the second to fourth units **10M**, **10C**, and **10K**, and the toner images of the respective colors are superimposed and transferred in a multiple manner.

The intermediate transfer belt **20** onto which the toner images of four colors are transferred in a multiple manner through the first to fourth units arrives at a secondary transfer unit including the intermediate transfer belt **20**, the support roller **24** in contact with the inner surface of the intermediate transfer belt, and a secondary transfer roller **26** (an example of the secondary transfer unit) disposed on the image carrying surface side of the intermediate transfer belt **20**. On the other hand, recording paper **P** (an example of the recording medium) is fed through a supply mechanism into a gap where the secondary transfer roller **26** and the intermediate transfer belt **20** are in contact with each other at a predetermined timing, and a secondary transfer bias is applied to the support roller **24**. The transfer bias applied at this time has the same polarity (-) as the toner polarity (-). The electrostatic force from the intermediate transfer belt **20** to the recording paper **P** acts on the toner image, and the toner image on the intermediate transfer belt **20** is transferred onto the recording paper **P**. The secondary transfer bias at this time is determined according to the resistance detected by a resistance detection unit (not illustrated) for detecting the resistance of the secondary transfer unit, and is voltage-controlled.

Thereafter, the recording paper **P** is sent to a pressure contact portion (so-called nip portion) of a pair of fixing rollers in a fixing device **28** (an example of the fixing unit), the toner image is fixed on the recording paper **P**, and a fixed image is formed.

Examples of the recording paper **P** onto which the toner image is transferred include plain paper for use in electro-photographic copying machines and printers. As the recording medium, in addition to the recording paper **P**, an OHP sheet or the like may be used.

To further improve the smoothness of the image surface after fixing, the surface of the recording paper **P** is also preferably smooth. For example, coated paper obtained by coating the surface of plain paper with a resin or the like, art paper for printing, and the like are preferably used.

The recording paper **P**, on which the fixing of the color image is completed, is conveyed out toward a discharge unit, and a series of color image forming operations is completed.

## &lt;Process Cartridge&gt;

The process cartridge according to the exemplary embodiment is a process cartridge which includes a developing unit for storing the electrostatic charge image developer according to the exemplary embodiment and for developing, as a toner image, the electrostatic charge image formed on the surface of the image carrier by using the electrostatic charge image developer, and which is attached to and detached from the image forming apparatus.

The process cartridge according to the exemplary embodiment is not limited to the above configuration and may be configured to include a developing unit and, if necessary, at least one selected from other units such as an image carrier, a charging unit, an electrostatic charge image forming unit, and a transfer unit.

Hereinafter, an example of the process cartridge according to the exemplary embodiment will be shown, but the process cartridge is not limited thereto. In the following description, the main parts shown in the drawings will be described, and description of the other parts will be omitted.

FIG. 2 is a schematic configuration diagram illustrating the process cartridge according to the exemplary embodiment. A process cartridge 200 illustrated in FIG. 2 is configured as a cartridge by, for example, integrally combining and holding a photoconductor 107 (an example of the image carrier), a charging roller 108 (an example of the charging unit) provided around the photoconductor 107, a developing device 111 (an example of the developing unit), and a photoconductor cleaning device 113 (an example of the cleaning unit) by a housing 117 provided with a mounting rail 116 and an opening 118 for exposure.

In FIG. 2, 109 denotes an exposure device (an example of the electrostatic charge image forming unit), 112 denotes a transfer device (an example of the transfer unit), 115 denotes a fixing device (an example of the fixing unit), and 300 denotes recording paper (an example of the recording medium).

## Examples

Hereinafter, the exemplary embodiment of the invention will be described in detail with reference to Examples, but the exemplary embodiment of the invention is not limited to these Examples. In the following description, the "parts" and "%" are based on mass unless otherwise specified.

## &lt;Preparation of Toner&gt;

## [Preparation of Amorphous Polyester Resin Dispersion Liquid (A1)]

Ethylene glycol: 37 parts

Neopentyl glycol: 65 parts

1,9-nonanediol: 32 parts

Terephthalic acid: 96 parts

The above materials are charged into a flask, the temperature is raised to 200°C. over 1 hour, and after confirming that the reaction system is uniformly stirred, 1.2 parts of dibutyltin oxide is charged thereto. While distilling off the produced water, the temperature is raised to 240°C. over 6 hours and stirring is continued at 240°C. for 4 hours, to obtain an amorphous polyester resin (acid value: 9.4 mg KOH/g, weight average molecular weight: 13,000, glass transition temperature: 62°C.). The amorphous polyester resin in the molten state is transported to an emulsifying disperser (Cavitron CD1010, manufactured by Eurotech Corporation) at a rate of 100 g/min. Separately, dilute ammonia water having a concentration of 0.37%, obtained by diluting reagent ammonia water with ion-exchanged water, is charged into a tank, and transported to the emul-

sifying disperser at the same time as the amorphous polyester resin at a rate of 0.1 l/min, while being heated to 120°C. with a heat exchanger. The emulsifying disperser is operated under the conditions of a rotor rotation speed of 60 Hz and a pressure of 5 kg/cm<sup>2</sup>, to obtain an amorphous polyester resin dispersion liquid (A1) having a volume average particle diameter of 160 nm and a solid content of 20%.

## [Preparation of Crystalline Polyester Resin Dispersion Liquid (C1)]

Decanedioic acid: 81 parts

Hexanediol: 47 parts

The above materials are charged into a flask, the temperature is raised to 160°C. over 1 hour, and after confirming that the reaction system is uniformly stirred, 0.03 part of dibutyltin oxide is charged thereto. While distilling off the produced water, the temperature is raised to 200°C. over 6 hours and stirring is continued at 200°C. for 4 hours. Then, the reaction liquid is cooled and subjected to solid-liquid separation, and the solid is dried at a temperature of 40°C. under reduced pressure, to obtain a crystalline polyester resin (C1) (melting point: 64°C., weight average molecular weight: 15,000)

Crystalline polyester resin (C1): 50 parts

Anionic surfactant (Neogen RK manufactured by DKS Co. Ltd.): 2 parts

Ion-exchanged water: 200 parts

The above materials are heated to 120°C., and dispersed using a (Ultra Turrax T50, manufactured by IKA Company), and then a dispersion treatment is performed using a pressure discharge homogenizer. When the volume average particle diameter reached 180 nm, the particles are collected to obtain a crystalline polyester resin dispersion liquid (C1) having a solid content of 20%.

## [Preparation of Release Agent Particle Dispersion Liquid (W1)]

Paraffin wax (HNP-9 manufactured by Nippon Seiro Co., Ltd.): 100 parts

Anionic surfactant (Neogen RK manufactured by DKS Co. Ltd.): 1 part

Ion-exchanged water: 350 parts

The above materials are mixed, heated to 100°C., and dispersed using a homogenizer (Ultra Turrax T50, manufactured by IKA Company), and then a dispersion treatment is performed using a pressure discharge Gaulin homogenizer, to obtain a release agent particle dispersion liquid in which release agent particles having a volume average particle diameter of 200 nm are dispersed. Ion-exchanged water is added to the release agent particle dispersion liquid to adjust the solid content to 20% to obtain a release agent particle dispersion liquid (W1).

## [Preparation of Colorant Particle Dispersion Liquid (C1)]

Cyan pigment (Pigment Blue 15:3 manufactured by Dainichiseika Color & Chemicals Mfg. Co., Ltd.): 50 parts

Anionic surfactant (Neogen RK manufactured by DKS Co. Ltd.): 5 parts

Ion-exchanged water: 195 parts

The above materials are mixed and subjected to a dispersion treatment for 60 minutes using a high-pressure impact disperser (Ultimizer HJP30006, manufactured by Sugino Machine Co., Ltd), to obtain a colorant particle dispersion liquid (C1) having a solid content of 20%.

## [Preparation of Cyan Toner Particles (C1)]

Ion-exchanged water: 200 parts

Amorphous polyester resin dispersion liquid (A1): 150 parts

Crystalline polyester resin dispersion liquid (C1): 10 parts

Release agent particle dispersion liquid (W1): 10 parts  
Colorant particle dispersion liquid (C1): 15 parts

Anionic surfactant (TaycaPower): 2.8 parts

The above materials are charged into a round stainless steel flask, 0.1 N nitric acid is added to adjust the pH to 3.5, and then a polyaluminum chloride aqueous solution prepared by dissolving 2 parts of polyaluminum chloride (manufactured by Oji Paper Company, 30% powder) in 30 parts of ion-exchanged water is added thereto. The mixture is dispersed at 30° C. using a homogenizer (Ultra Turrax T50, manufactured by IKA Company), and then heated to 45° C. in a heating oil bath and kept until the volume average particle diameter becomes 4.9  $\mu\text{m}$ . Then, 60 parts of the amorphous polyester resin dispersion liquid (A1) is added and held for 30 minutes. Then, when the volume average particle diameter reaches 5.2  $\mu\text{m}$ , 60 parts of the amorphous polyester resin dispersion liquid (A1) is further added and held for 30 minutes. Subsequently, 20 parts of 10% NTA (nitrilotriacetate) metal salt aqueous solution (CHIREST 70, manufactured by CHIREST Corporation) is added, and a 1 N sodium hydroxide aqueous solution is added to adjust the pH to 9.0. Then, 1 part of an anionic surfactant (TaycaPower) is charged thereto, and the mixture is heated to 85° C. and held for 5 hours while continuing stirring. Then, the mixture is cooled to 20° C. at a rate of 20° C./min. Then, the mixture is filtered, washed thoroughly with ion-exchanged water, and dried, to obtain cyan toner particles (C1) having a volume average particle diameter of 5.5  $\mu\text{m}$ .

[Preparation of Cyan Toner (C1)]

100 parts by mass of the cyan toner particles (C1) and 1.5 parts by mass of hydrophobic silica particles (RY50, manufactured by Nippon Aerosil Co., Ltd.) are charged into a sample mill and mixed at a rotation speed of 10,000 rpm for 30 seconds. Then, the mixture is sieved with a vibrating sieve having an opening of 45  $\mu\text{m}$  to obtain a cyan toner (C1) having a volume average particle diameter of 5.5  $\mu\text{m}$ .

<Preparation of Silica Particles>

The following silica particles are prepared.

Silica particles (1): hydrophobic silica particles surface-treated with hexamethyldisilazane, volume average particle diameter of primary particles: 4 nm, monodispersed.

Silica particles (2): hydrophobic silica particles surface-treated with hexamethyldisilazane, volume average particle diameter of primary particles: 7 nm, monodispersed.

Silica particles (3): hydrophobic silica particles surface-treated with hexamethyldisilazane, volume average particle diameter of primary particles: 12 nm, monodispersed.

Silica particles (4): hydrophobic silica particles surface-treated with hexamethyldisilazane, volume average particle diameter of primary particles: 35 nm, monodispersed.

Silica particles (5): hydrophobic silica particles surface-treated with hexamethyldisilazane, volume average particle diameter of primary particles: 65 nm, monodispersed.

Silica particles (6): hydrophobic silica particles surface-treated with hexamethyldisilazane, volume average particle diameter of primary particles: 85 nm, monodispersed.

Silica particles (7): hydrophobic silica particles surface-treated with hexamethyldisilazane, volume average particle diameter of primary particles: 93 nm, monodispersed.

<Preparation of Resin-Coated Carrier>

[Carrier (1)]

Mg ferrite core material (volume average particle diameter: 35  $\mu\text{m}$ ): 100 parts

5 Resin particles of styrene-methyl methacrylate copolymer (polymerization ratio based on mass: 2/8, weight average molecular weight: 500,000): 3.5 parts

Silica particles (1): 0.7 part

The above materials are charged into a stirring mixer with stirring blades, the temperature inside the stirring mixer is set to 20° C., and the mixture is stirred and mixed for 15 minutes at a peripheral speed of the stirring blades of 11.0 m/s (first stirring step), to adhere the resin particles and the silica particles to the core material.

10 Then, the temperature in the stirring mixer is set to 140° C., and the mixture is stirred and mixed for 10 minutes at a peripheral speed of the stirring blades of 7.0 m/s (second stirring step).

15 The powder is taken out from the stirring mixer, and the coarse powder is removed by sieving with a mesh having an opening of 75  $\mu\text{m}$  to obtain a carrier (1).

[Carriers (2) to (7)]

20 Carriers (2) to (7) are obtained in the same manner as the preparation of the carrier (1), except that the silica particles (1) are changed to the corresponding silica particles (2) to (7).

[Carriers (8) to (19)]

25 Carriers (8) to (19) are obtained in the same manner as the preparation of the carrier (4), except that the first stirring step and the second stirring step are changed as shown in Table 1.

[Carriers (20) and (21)]

30 Carriers (20) and (21) are obtained in the same manner as the preparation of the carrier (4), except that the amounts of the resin particles and the silica particles added are increased or decreased, and the first stirring step and the second stirring step are changed as shown in Table 1.

[Carrier (22)]

35 Cyclohexyl methacrylate resin (weight average molecular weight: 50,000): 20 parts

Silica particles (4): 20 parts

Toluene: 250 parts

Methanol: 50 parts

40 The above materials and glass beads (diameter: 1 mm, the same amount as toluene) are charged into a sand mill and stirred at a rotation speed of 190 rpm for 30 minutes, to obtain a coating agent (1).

45 1,000 parts of the Mg ferrite core material (volume average particle diameter: 35  $\mu\text{m}$ ) and 125 parts of the coating agent (1) are charged into a kneader and mixed at room temperature (25° C.) for 20 minutes. Then, the mixture is heated to 70° C. and dried under reduced pressure.

50 The dried product is cooled to room temperature (25° C.), 55 125 parts of the coating agent (1) is additionally added, and the mixture is mixed at room temperature (25° C.) for 20 minutes. Then, the mixture is heated to 70° C. and dried under reduced pressure.

56 Then, the dried product is taken out from the kneader, and the coarse powder is removed by sieving with a mesh having an opening of 75  $\mu\text{m}$  to obtain a carrier (22).

[Carriers (23) and (24)]

60 Carriers (23) and (24) are obtained in the same manner as the preparation of the carrier (22), except that the drying treatment of heating to 70° C. and depressurizing in the kneader is repeated until the amount of toluene reaches a desired content.

## &lt;Preparation of Developer&gt;

The corresponding carriers (1) to (24) and the cyan toner (C1) are charged in a V blender at a mixing ratio of carrier:toner=100:8 (mass ratio) and stirred for 20 minutes, to obtain cyan developers (K1) to (K24).

## &lt;Measurement of Average Particle Diameter of Silica Particles in Resin Layer&gt;

The carrier is embedded in an epoxy resin and cut with a microtome to prepare a carrier cross section. An SEM image of the carrier cross section taken by a scanning transmission electron microscope (S-4100 manufactured by Hitachi, Ltd.) is taken into an image processing analysis device (Luzex AP manufactured by Nireco) to perform image analysis. 100 silica particles (primary particles) in the resin layer are randomly selected, a circle-equivalent diameter (nm) of each particle is determined, and the circle-equivalent diameters are arithmetically averaged to obtain the average particle diameter (nm) of the silica particles.

## &lt;Measurement of Average Thickness of Resin Layer&gt;

The SEM image is taken into an image processing analysis device (Luzex AP manufactured by Nireco) to perform image analysis. The thickness ( $\mu\text{m}$ ) of the resin layer is measured by randomly selecting 10 points per one particle of the carrier, 100 carriers are further measured, and the thicknesses are arithmetically averaged to obtain the average thickness ( $\mu\text{m}$ ) of the resin layer.

## &lt;Carrier Surface Analysis&gt;

As a device for three-dimensionally analyzing the surface of the carrier, an electron beam three-dimensional roughness analyzer ERA-8900FE manufactured by Elionix Inc. is used. The carrier surface analysis performed by ERA-8900FE is specifically performed as follows.

The surface of one carrier particle is enlarged to 5000 times, three-dimensional measurement is performed by taking 400 measurement points in the long side direction and 300 measurement points in the short side direction, and a region of  $24 \mu\text{m} \times 18 \mu\text{m}$  is measured to obtain three-dimensional image data. For the three-dimensional image data, the limit wavelength of the spline filter is set to  $12 \mu\text{m}$  to remove wavelengths having a period of  $12 \mu\text{m}$  or more, and the cutoff value of the Gaussian high-pass filter is set to  $2.0 \mu\text{m}$  to remove wavelengths having a period of  $2.0 \mu\text{m}$  or more, so as to obtain three-dimensional roughness curve data. From the three-dimensional roughness curve data, the surface area B ( $\mu\text{m}^2$ ) of a central region of  $12 \mu\text{m} \times 12 \mu\text{m}$  (plan view area A= $144 \mu\text{m}^2$ ) is obtained to obtain the ratio B/A. The ratio B/A is calculated for 100 carriers and arithmetically averaged.

## &lt;Measurement of Exposed Area Ratio of Magnetic Particles on Carrier Surface&gt;

The carrier is used as a sample and analyzed by X-ray photoelectron spectroscopy (XPS) under the following conditions, to obtain the exposed area ratio (%) of the magnetic particles.

XPS device: VersaProbeII, manufactured by ULVAC-PHI, INCORPORATED

Etching gun: argon gun

Accelerating voltage: 5 kV

Emission current: 20 mA

Sputter region: 2.0 mm  $\times$  2.0 mm

Sputter rate: 3 nm/min

## &lt;Measurement of Amount of Toluene in Carrier&gt;

1 g of a carrier within 24 hours after production is weighed and added to 20 mL of chloroform to dissolve a resin forming the resin layer. Then, 5 mL of methanol is added thereto, and the mixture is left in a sealed container for one day. The supernatant liquid after standing is used as a

sample, gas chromatography mass spectrometry is performed under the following conditions.

Gas chromatograph mass spectrometer: 263-50, manufactured by Hitachi, Ltd.

Column: TC-17 manufactured by GL Science Inc. (inner diameter: 0.32 mm, length: 30 m, liquid phase: 0.25  $\mu\text{m}$ )

Column temperature: 40° C. (5 minutes)  $\rightarrow$  (5° C./minute)  $\rightarrow$  80° C. (2 minutes)

Inlet temperature: 200° C.

Splitless injection method, purge time: 30 seconds

Carrier gas type: helium

Carrier gas pressure: 35 kPa

A calibration curve is prepared using a standard solution in which the concentration is changed by diluting toluene with methanol. The amount of toluene is obtained from the peak area of toluene that appeared in the chromatograph of the sample and the calibration curve of the standard substance. Then, the amount of toluene (ppm) based on the total amount of the carrier is calculated.

## &lt;Evaluation on Change in Image Density&gt;

A modified machine of an image forming apparatus DocuCenterColor400 (manufactured by Fuji Xerox Co., Ltd.) is prepared, and the corresponding developers (1) to (4) are changed into a developing machine. The image forming apparatus is left under an environment of a temperature of 10° C. and a relative humidity of 15% for 24 hours. Under the environment of temperature of 10° C. and a relative humidity of 15%, 50,000 test charts with an image density of 5% are continuously output to A4 size plain paper. The L\* value, a\* value, and b\* value are measured at 3 points on each of the 1,000th image and the 50,000th image by using a spectrophotometer (X-Rite Ci62, manufactured by X-Rite Inc.). The color difference  $\Delta E$  is calculated based on the following equation, and the color difference  $\Delta E$  is classified as follows.

$$\Delta E = \sqrt{(L_1 - L_2)^2 + (a_1 - a_2)^2 + (b_1 - b_2)^2}$$

In the equation,  $L_1$ ,  $a_1$  and  $b_1$  are the L\* value, the a\* value and the b\* value of the 1,000th image (the average value at the 3 points), and  $L_2$ ,  $a_2$ , and  $b_2$  are the L\* value, the a\* value, and the b\* value of the 50,000th image (the average value at the 3 points).

G0: Color difference  $\Delta E$  is 1 or less. G1: Color difference  $\Delta E$  is more than 1 and 3 or less. G2: Color difference  $\Delta E$  is more than 3 and 5 or less. G3: Color difference  $\Delta E$  is more than 5.

The foregoing description of the exemplary embodiments of the present invention has been provided for the purposes of illustration and description. It is not intended to be exhaustive or to limit the invention to the precise forms disclosed. Obviously, many modifications and variations will be apparent to practitioners skilled in the art. The embodiments were chosen and described in order to best explain the principles of the invention and its practical applications, thereby enabling others skilled in the art to understand the invention for various embodiments and with the various modifications as are suited to the particular use contemplated. It is intended that the scope of the invention be defined by the following claims and their equivalents.

TABLE 1

| Developer             | Carrier | Silica particles | Resin layer         |                                              |            |                      |                        |            |                                                    |                        |           |                                      |                         |                         |    |
|-----------------------|---------|------------------|---------------------|----------------------------------------------|------------|----------------------|------------------------|------------|----------------------------------------------------|------------------------|-----------|--------------------------------------|-------------------------|-------------------------|----|
|                       |         |                  | First stirring step |                                              |            | Second stirring step |                        |            | Average particle diameter [nm] of silica particles | Average thickness [μm] | Ratio B/A | Exposed                              |                         |                         |    |
|                       |         |                  | Temperature [°C.]   | Peripheral speed [m/s]                       | Time [min] | Temperature [°C.]    | Peripheral speed [m/s] | Time [min] |                                                    |                        |           | area ratio [%] of magnetic particles | Amount [ppm] of toluene | Change in image density |    |
| Comparative Example 1 | (1)     | (1)              | (1)                 | 20                                           | 11.0       | 15                   | 140                    | 7.0        | 10                                                 | 4                      | 0.9       | 1.050                                | 0.9                     | 0                       | G3 |
| Example 1             | (2)     | (2)              | (2)                 | 20                                           | 11.0       | 15                   | 140                    | 7.0        | 10                                                 | 7                      | 0.7       | 1.042                                | 1.7                     | 0                       | G2 |
| Example 2             | (3)     | (3)              | (3)                 | 20                                           | 11.0       | 15                   | 140                    | 7.0        | 10                                                 | 12                     | 1.0       | 1.044                                | 1.2                     | 0                       | G1 |
| Example 3             | (4)     | (4)              | (4)                 | 20                                           | 11.0       | 15                   | 140                    | 7.0        | 10                                                 | 35                     | 1.1       | 1.055                                | 1.7                     | 0                       | G0 |
| Example 4             | (5)     | (5)              | (5)                 | 20                                           | 11.0       | 15                   | 140                    | 7.0        | 10                                                 | 65                     | 1.1       | 1.050                                | 2.5                     | 0                       | G1 |
| Example 5             | (6)     | (6)              | (6)                 | 20                                           | 11.0       | 15                   | 140                    | 7.0        | 10                                                 | 85                     | 0.9       | 1.049                                | 1.9                     | 0                       | G2 |
| Comparative Example 2 | (7)     | (7)              | (7)                 | 20                                           | 11.0       | 15                   | 140                    | 7.0        | 10                                                 | 93                     | 1.2       | 1.061                                | 3.2                     | 0                       | G3 |
| Comparative Example 3 | (8)     | (8)              | (4)                 | 20                                           | 11.0       | 15                   | 140                    | 5.0        | 28                                                 | 35                     | 0.8       | 1.019                                | 2.3                     | 0                       | G3 |
| Example 6             | (9)     | (9)              | (4)                 | 20                                           | 11.0       | 15                   | 140                    | 5.0        | 25                                                 | 35                     | 1.0       | 1.021                                | 2.2                     | 0                       | G2 |
| Example 7             | (10)    | (10)             | (4)                 | 20                                           | 11.0       | 15                   | 140                    | 3.0        | 15                                                 | 35                     | 1.1       | 1.047                                | 2.5                     | 0                       | G1 |
| Example 8             | (11)    | (11)             | (4)                 | 20                                           | 11.0       | 15                   | 120                    | 3.0        | 10                                                 | 35                     | 1.0       | 1.063                                | 1.2                     | 0                       | G0 |
| Example 9             | (12)    | (12)             | (4)                 | 20                                           | 11.0       | 15                   | 120                    | 3.0        | 7                                                  | 35                     | 1.1       | 1.099                                | 1.5                     | 0                       | G2 |
| Comparative Example 4 | (13)    | (13)             | (4)                 | 20                                           | 11.0       | 15                   | 140                    | 3.0        | 5                                                  | 35                     | 1.0       | 1.101                                | 0.9                     | 0                       | G3 |
| Comparative Example 5 | (14)    | (14)             | (4)                 | 20                                           | 5.0        | 15                   | 140                    | 3.0        | 3                                                  | 35                     | 1.2       | 1.062                                | 0.04                    | 0                       | G3 |
| Example 10            | (15)    | (15)             | (4)                 | 20                                           | 5.0        | 15                   | 140                    | 3.0        | 5                                                  | 35                     | 1.0       | 1.059                                | 0.11                    | 0                       | G2 |
| Example 11            | (16)    | (16)             | (4)                 | 20                                           | 11.0       | 15                   | 140                    | 5.0        | 10                                                 | 35                     | 1.1       | 1.049                                | 1.4                     | 0                       | G1 |
| Example 12            | (17)    | (17)             | (4)                 | 20                                           | 11.0       | 15                   | 140                    | 10.0       | 10                                                 | 35                     | 1.0       | 1.044                                | 2.1                     | 0                       | G1 |
| Example 13            | (18)    | (18)             | (4)                 | 20                                           | 20.0       | 20                   | 170                    | 12.0       | 14                                                 | 35                     | 1.0       | 1.031                                | 3.9                     | 0                       | G2 |
| Comparative Example 6 | (19)    | (19)             | (4)                 | 20                                           | 20.0       | 20                   | 170                    | 12.0       | 20                                                 | 35                     | 0.7       | 1.040                                | 5.0                     | 0                       | G3 |
| Example 14            | (20)    | (20)             | (4)                 | 20                                           | 5.0        | 15                   | 160                    | 5.0        | 10                                                 | 35                     | 0.6       | 1.052                                | 3.0                     | 0                       | G2 |
| Example 15            | (21)    | (21)             | (4)                 | 20                                           | 50.0       | 15                   | 140                    | 5.0        | 20                                                 | 35                     | 1.4       | 1.046                                | 1.0                     | 0                       | G1 |
| Example 16            | (22)    | (22)             | (4)                 | Forming resin layer by wet production method |            |                      |                        |            | 35                                                 | 1.2                    | 1.056     | 2.2                                  | 200                     | G2                      |    |
| Example 17            | (23)    | (23)             | (4)                 | Forming resin layer by wet production method |            |                      |                        |            | 35                                                 | 1.1                    | 1.056     | 3.3                                  | 80                      | G1                      |    |
| Example 18            | (24)    | (24)             | (4)                 | Forming resin layer by wet production method |            |                      |                        |            | 35                                                 | 1.2                    | 1.056     | 2.9                                  | 15                      | G0                      |    |

What is claimed is:

- An electrostatic charge image developing carrier comprising:  
magnetic particles; and  
an acrylate resin layer coating the magnetic particles and  
containing silica particles,  
wherein an exposed area ratio of the magnetic particles is  
0.1% or more and 4.0% or less,  
wherein an average particle diameter of the silica particles is  
5 nm or more and 90 nm or less, and  
wherein a ratio B/A of a surface area B of the electrostatic  
charge image developing carrier to a plan view area A  
of the electrostatic charge image developing carrier is  
1.020 or more and 1.100 or less when a surface of the  
electrostatic charge image developing carrier is three-  
dimensionally analyzed.
- The electrostatic charge image developing carrier  
according to claim 1, wherein the ratio B/A is 1.040 or more  
and 1.080 or less.
- The electrostatic charge image developing carrier  
according to claim 1, wherein the average particle diameter of  
the silica particles is 5 nm or more and 70 nm or less.
- The electrostatic charge image developing carrier  
according to claim 1, wherein the exposed area ratio of the  
magnetic particles is 0.3% or more and 3.5% or less.
- The electrostatic charge image developing carrier  
according to claim 1, wherein an average thickness of the  
resin layer is 0.6 μm or more and 1.4 μm or less.
- The electrostatic charge image developing carrier  
according to claim 5, wherein the average thickness of the  
resin layer is 0.8 μm or more and 1.2 μm or less.
- The electrostatic charge image developing carrier  
according to claim 1, wherein an amount of toluene in the  
electrostatic charge image developing carrier is 100 ppm or  
less.
- The electrostatic charge image developing carrier  
according to claim 7, wherein the amount of toluene in the  
electrostatic charge image developing carrier is 20 ppm or  
less.
- An electrostatic charge image developer comprising:  
the electrostatic charge image developing carrier according  
to claim 1; and  
an electrostatic charge image developing toner.
- An image forming apparatus comprising:  
an image carrier;  
a charging unit configured to charge a surface of the  
image carrier;  
an electrostatic charge image forming unit configured to  
form an electrostatic charge image on the surface of the  
charged image carrier;  
a developing unit configured to develop the electrostatic  
charge image formed on the surface of the image carrier  
as a toner image by the electrostatic charge image  
developer according to claim 9;  
a transfer unit configured to transfer the toner image onto  
a surface of a recording medium; and  
a fixing unit configured to fix the transferred toner image  
onto the surface of the recording medium.
- The electrostatic charge image developing carrier  
according to claim 1,  
wherein a volume average particle diameter of the mag-  
netic particles is 15 μm or more and 100 μm or less.

12. The electrostatic charge image developing carrier according to claim 1, wherein the electrostatic charge image developing carrier is a resin-coated carrier.

\* \* \* \* \*